

**C. CRAWFORD.**  
**PROCESS FOR CASTING MOLTEN METAL IN MOLDS.**  
**APPLICATION FILED JUNE 14, 1909.**

1,040,517.

Patented Oct. 8, 1912.



WITNESSES.  
Charles R. Sprague  
Geo. F. Colby

# UNITED STATES PATENT OFFICE.

CLAY CRAWFORD, OF TOLEDO, OHIO, ASSIGNEE TO O. S. BRIGHAM, OF TOLEDO, OHIO.

## PROCESS FOR CASTING MOLTEN METAL IN MOLDS.

1,040,517.

Specification of Letters Patent.

Patented Oct. 8, 1912.

Application filed June 14, 1909. Serial No. 502,170.

*To all whom it may concern:*

Be it known that I, CLAY CRAWFORD, a citizen of the United States, residing at 845 West Woodruff avenue, in the city of Toledo, county of Lucas, and State of Ohio, have invented new and useful Improvements in Processes for Casting Molten Metal in Molds, of which the following is a specification.

- 10 This invention relates to the process of casting molten metal in molds and has for its object: First. The separation and elimination of the contained slags, segregates and gases, which cause flaws and other defects. 15 Second. Also to break up the axes and planes of cleavage in the forming crystals, which weaken the resulting casting. Third. To form and retain to the end of the solidifying period a feeding head to reduce or 20 prevent piping, or a honeycombed core along the central axis of the casting.

I shall describe my invention with reference to the accompanying drawing of a machine for casting steel ingots by this process.

25 The machine used herein for illustration is the subject of an application for a patent now pending, filed October 21st, 1907, Number 398,498, but which can be used for many other forms of castings.

30 It consists of a mold mounted on a table, supported on the top end of a vertical shaft, with means to rotate the mold about its vertical axis, with a constantly varying speed of rotation, coöoperating simultaneously, 35 with means to accelerate the cooling of the lower portion of the mold and casting, and to retard the cooling of the upper portion.

Among engineers it is a well known fact 40 that metal castings, especially of steel, are not perfectly homogeneous and their reliability and value is much reduced by these defects. During all the time the liquid metal is cooling there are processes going on by which the carbon, phosphorus, slags and 45 sulfur are being segregated, and the segregates concentrated in the central portion of the mass, and being lighter than the molten metal, most of them rise to the upper portion or surface of the core of molten metal.

50 In the manufacture of steel as now conducted, a portion of the upper end of the ingots are cut off and scrapped, causing a great loss of material, but even then the central portion of what is left is not uniform 55 with the outside portion, and contains slags,

segregates, blowholes, and holes caused by the solidification of an outside shell and the shrinkage of the inner portion as it cools, leaving a honeycombed core. Rolling or hammering while the ingot is highly heated 60 partially remedies some of these defects but not wholly so.

The process by which I reduce or eliminate the defects in the cast shapes to which it is applicable, is to oscillate or rotate with 65 a constantly varying speed of rotation, the mold about its vertical axis, and at the same time regulate the cooling of the molten metal, so that the solidification shall proceed progressively from the bottom and 70 sides of the mold and ending at the center of the upper surface. This leaves an avenue open for the escape of impurities, as they concentrate in the center and rise to the surface, if not prevented by the upper portion 75 solidifying. This also gives a "feeding head" to supply metal to correct the shrinkage due to solidification. The rotation of the mold about its vertical axis, with a constantly varying speed of rotation, causes 80 every particle of the liquid metal to slide over the surface of every adjacent particle, which agitation separates the impurities and they rise to the upper surface of the core of liquid metal, and they can afterward be 85 separated by cutting them off the upper end of the ingot. The mold may be oscillated about its vertical axis to get the same effect as rotation with a constantly varying rotative velocity. A box shaped mold may be 90 mounted on rollers and oscillated or shaken in a horizontal plane with the cooling of the top portion retarded, and the cooling of the bottom portion accelerated, to get the same effect as by rotation with a constantly 95 varying rotative velocity. In other words, the process in its broadest aspect may be said to consist in agitating a body of molten metal during the cooling of the same. Such agitation causing the unfrozen or molten metal to move or slide over the surface of that portion of the metal which has already solidified. More specifically, the process includes the production of the agitating movement by moving the metal to be cast 100 with varying or unequal velocities in equal intervals of time.

It is a law of the molecular aggregation of crystalline solids that when their particles consolidate under the influence of heat and 110

motion; their crystals arrange and group themselves with their principal axes in lines perpendicular to the cooling surfaces of the solids. In castings of rectangular section these axes meet at points equidistant from the cooling surfaces, and are there imperfectly connected and form a core or seam, which will contain a varying amount of slag or other impurities, which form a cleavage plane that is easy to rupture, and which it is impossible to remove by subsequent working with rolls or hammers. This form of crystallization is nicely shown in a cake of artificial ice. In molds of circular cross section there is apt to be a flow of impurities to the center of the ingot, forming a vertical core or pipe. My process of constantly sliding the liquid metal over the surfaces of the solidified metal breaks up the axes of crystallization, and at the same time separates the impurities, which rise to the surface and gives much stronger castings, free from coarse planes of cleavage, and better adapted to after treatment with rolls and hammer.

Reference should be had to the accompanying drawings forming a part of this specification in which—

Figure 1 is a front elevation of the mechanism for rotating the mold; Fig. 2 is an end elevation of the mechanism for rotating the mold; and Fig. 3 is a front elevation, partly in section, of the mold and apparatus for rotating the same.

Referring to the accompanying drawing, 1 is the frame of the machine, 2 is a hollow, vertical shaft, supported by frame 1, and having secured on its upper end a table 3, which has a flange extending from its outer circumference; resting on table 3 is a plate 15, which forms a bottom for the ingot mold 16. A portion of the upper end of the ingot mold may be enlarged and lined with a belt 17 of a non-conductor of heat to prevent radiation of heat and retard the cooling of the liquid metal 19, and 18 is a covering of a non-conductor of heat on the upper surface of the molten metal to prevent the radiation of heat from the upper surface of the liquid metal, and retard the solidification of the surface of the metal to the very last end of the cooling process.

20 is metal that has solidified around the sides and bottom of the mold.

21 are pipes that may be used to throw jets from holes 22 of a cooling fluid (as a mist of air and water) on the lower and outer surface of the mold, to accelerate the cooling of the metal in that portion of the mold. These jets are so controlled that each 60 ring may be applied progressively from the lower to the upper ring of jets.

23 are thin ribs integral with the mold and projecting from its sides at its lower end with the upper end gradually merging 65 into the outer surface of the mold as they

rise. The ribs furnish radiating surface for the purpose of accelerating the cooling of the contained metal at its lower end.

Instead of lining 17, a belt of a non-conductor of heat may be used to cover the outer surface of the upper end of the mold to obtain the same results as those obtained by lining 17.

On the vertical shaft 2 is a beveled gear 4 meshing into gear 5 on shaft 7, supported by bearings 6; on shaft 7 is crank 8, having a pin 9, on which is box 10, sliding in a slot in crank 11, on the end of shaft 13, which is turned by a belt on pulley 14. The shafts 7 and 13 are parallel, but not in the same line, 75 13 being shown a little higher than 7, and as they rotate with a mean angular velocity the angular velocity ratio at each instant is varying; in the position shown the angular velocity of gear 4 would be at a minimum, 80 and with the cranks pointing downward it would be at its maximum velocity.

The mode of operation is to rotate the table and mold with a constantly varying speed of rotation, then fill the mold with 90 molten metal from a ladle in the usual manner, then cover the upper surface of the molten metal with a non-conductor of heat, as air-slaked lime, to prevent the radiation of heat as much as possible, then, if necessary, apply the cooling fluid from the lowest ring of jets and progressively at intervals to the upper ring of jets as may be needed to cool the metal progressively from the bottom upward. The effect of this process of retarding the cooling of the upper end of the casting and the accelerating the cooling of its lower end soon forms the shell 20 of solidified steel next the bottom sides of the mold, with the sides of the shell 20 decreasing gradually in thickness toward the top portion, and during the process of cooling there will be a core 19 of molten metal of inverted conoidal shape, which will constantly decrease in size as the cooling proceeds, until it finally disappears at the center of the top of the casting. The center of the extreme top surface being the last point to solidify.

One of the most important points of my process is to keep the top of the molten metal liquid to the end of the solidifying stage, and thus to furnish a feeder to fill up the space left in the interior of the casting due to the shrinkage of the contained cooling metal, this liquid core also furnishes an outlet for the contained slags, segregates and gases to escape out through the upper surface of the molten metal. This rotating of the mold with a constantly varying speed of rotation keeps every particle of the molten metal moving over the surfaces of its adjacent particles, and the surface of the molten core 19 over the surface of the solidified metal 20 at the bottom and sides of the 125 130

casting. This sliding of the particles upon one another is caused by the resistance of their inertia to a change in their rotative velocity about the axis of rotation, and by 5 their friction on the surface of the solidified metal and on each other. This sliding and agitation separates the slags and nodular segregates and also the occluded gases, and as they are lighter than the molten metal, 10 they arise to its surface and separate from it. Also the agitation brings the particles of oxid of iron in the molten metal into contact with the carbon and it is reduced to metallic iron.

15 When castings are allowed to solidify on their upper surface while the interior is molten, shrinkage causes a honeycombed core in the interior, which in effect are flaws and cannot be eliminated by subsequent 20 hammering or rolling. I greatly reduce or eliminate this center by keeping the upper surface fluid, which also allows the escape of the gases, slags and segregates, and concentrates them at the upper surface 25 of the casting. This separation is greatly accelerated by oscillating or rotating with a constantly varying speed of rotation, the mold around its vertical axis.

30 Changes may be made in some of the minor details while the essential features are retained, and the spirit of the invention embodied.

Having described my invention and its general method of operation what I claim is:—

35 1. The process of casting, which consists in introducing the metal into a mold, causing the metal to cool more rapidly in one part of the mold than in the others and simultaneously causing the particles of the

unsolidified metal to move with respect to 40 each other and to the solidified metal during the cooling.

2. The process of casting, which consists in introducing the metal into a mold, cooling the mold progressively from one end toward 45 the opposite end thereof and simultaneously causing the particles of the unsolidified metal to move with respect to each other and to the solidified metal during the cooling.

3. The process of casting which consists in 50 rotating a body of molten metal within a mold, throughout a succession of time periods, the velocity of rotation of the mold varying during each time period.

4. The process of casting, which consists in 55 introducing the metal into a mold, subjecting the mold to rotary motion so that the same moves with unequal velocities in equal intervals of time and simultaneously cooling one portion of the mold more rapidly than the other portions.

5. The process of casting, which consists in 60 moving the body of metal with unequal velocities in equal intervals of time and simultaneously preventing the radiation of 65 heat from a certain portion of the metal and cooling another portion of the metal.

6. The process of casting, which consists in 70 introducing the metal into a mold, rotating the mold with unequal velocities in equal intervals of time and preventing the radiation of heat from the exposed surface of the metal.

CLAY CRAWFORD.

Witnesses:

CHARLES R. SPRAGUE,  
GEORGE P. KING.